

1,282,267.

M. M. MERRITT,  
GALVANOPLASTIC PROCESS AND PRODUCT "B."  
APPLICATION FILED NOV. 2, 1917.

Patented Oct. 22, 1918.



Inventor:  
Meredith M. Merritt.  
by Emery Booth Journeyc & Varney,  
Attns.

# UNITED STATES PATENT OFFICE.

MATTHEW M. MERRITT, OF SOUTH MIDDLETON, MASSACHUSETTS, ASSIGNOR TO COPPER PRODUCTS COMPANY, OF BOSTON, MASSACHUSETTS, A CORPORATION OF MAINE.

## GALVANOPLASTIC PROCESS AND PRODUCT "B."

1,282,267.

Specification of Letters Patent. Patented Oct. 22, 1918.

Application filed November 2, 1917. Serial No. 199,811.

*To all whom it may concern:*

Be it known that I, MATTHEW M. MERRITT, a citizen of the United States, and a resident of South Middleton, county of Essex, Commonwealth of Massachusetts, have invented an Improvement in Galvanoplastic Processes and Products "B," of which the following description, in connection with the accompanying drawings, is a specification, 10 like characters on the drawings representing like parts.

This invention pertains to improvements in galvanoplastic processes and products, but more particularly, though not exclusively, to the manufacture of articles such as manifolds for internal combustion engines such as aeroplane engines.

In the drawings, which show one form of an illustrative embodiment of my invention:

20 Figure 1 shows a manifold;

Fig. 2 is a diagrammatic section therethrough on the line 2—2 of Fig. 1.

Great difficulty has been experienced in constructing manifolds for aeroplane engines of the requisite light weight which are strong enough to withstand the constant and excessive vibrations occasioned by the operation of the engine. Such manifolds are very likely to develop cracks, particularly 30 adjacent the bent portions thereof. It has heretofore been attempted to manufacture such manifolds by the electrolytic deposit of copper on cathodes of metal fusible at a low temperature, and on cathodes of wax 35 painted with graphite or other electrically conductive material, the core being melted out after the electrolytic deposit. Manifolds made by the usual methods, above-described, have proved unsatisfactory because 40 of brittleness and coarseness of texture of the deposited metal, this brittleness being accentuated at points adjacent curved portions of the deposit.

I have found that the deposits made as before described are rendered more uniform in quality by intermittent immersion of the cathode, as by attaching the same to a revolving wheel partially immersed in the electrolyte so that the entire cathode or a 50 considerable portion thereof, preferably at least one-half, is only intermittently immersed in the electrolyte. This aspect of my invention is not claimed herein being comprised in the subject matter of a copending 55 application Serial No. 247,966, filed August

2, 1918. While intermittent immersion improves the texture of the deposited metal, electrolytic deposits made on metallic cathodes having low melting points are, as heretofore made, likely to be rough and 60 brittle. I believe this to be due to the tendency of certain ingredients of the fusible metal, which is usually an alloy of lead, to be attacked by the electrolyte, and in some instances to be disassociated into negative ions traveling from the cathode to the anode.

Where, on the other hand, the cathode is formed of non-conductive material removable by fusion, by a solvent, or otherwise, 70 and the surface of which is coated with an electrically conductive paint, such as graphite, bronze powder and the like, the deposited copper, as heretofore practised, has been brittle and of slight tensile strength. 75 As stated in my co-pending application, filed herewith, I believe this to be due to the comparatively coarse texture of the conductive coating which is necessarily full of interstices as compared with cast, rolled, or electrolytically deposited metal. The unevenness of attraction exerted by this surfacing of the cathode results in combining the deposited metal in relatively coarse crystalline formation, which renders it brittle and of 85 slight tensile strength.

I have found that the deleterious effects of a cathode composed of metal having a low fusing-point may be minimized by coating the metal with a film of a foreign substance such as grease, and that if a layer of copper, preferably relatively thin, be electrolytically deposited subsequent to the application of the grease and the surface of this metal be coated with grease, that subsequent electrolytic deposits on the greased surface will be of fine texture and of great tensile strength, the brittleness being greatly reduced, if not eliminated. If desired, the 90 structure may be laminated by the occasional interruption of electrolytic deposit and the application to the surface of the deposited metal of films of grease.

Where it is necessary or desirable to utilize a non-metallic cathode such as wax or any electrically non-conductive material removable by a solvent or otherwise, the same being coated with a paint of electrolytically conductive material, I have found it of great advantage to coat the surface of the 105 110

electrically conductive material or paint with a thin film of grease, to deposit a relatively thin sheet of copper or other metal on the greased surface and, if desired, to provide a laminated structure by subsequently occasionally interrupting the electrolytic deposit and applying grease to the surface of the deposited metal.

Throughout this application I have used 10 the word "grease" generically to define any substance capable of forming a film of electrically non-conductive material over the surface on which the metal is to be deposited.

15 After electro-deposition the core of the cathode may be removed by fusion, by burning, by the use of a solvent or any other suitable method.

I have utilized the word "galvanoplastic" 20 in its broader sense to include any electrolytic processes in which the entire cathode or any portion thereof is removed subsequent to electro-deposition.

It is obvious that the cathode may, if desired, be exterior to the surface thereof on 25 which metal is to be deposited, and that for some purposes my invention may be useful in connection with galvanoplastic processes in which the cathode can be withdrawn 30 without change in the structure thereof.

While I have shown and described one embodiment of my invention and one method of practising the same, it will be understood that major changes may be

made, both in the product and the method 35 of producing the same, without departing from the scope of my invention, which is best defined in the following claims.

Claims:

1. A manifold comprising a tubular portion 40 formed of a plurality of layers of electrolytically deposited metal with a film of grease interposed between said layers.

2. A manifold comprising a tubular portion 45 formed of a plurality of layers of electrolytically deposited metal with non-conductive material interposed between said layers.

3. A manifold comprising a tubular portion 50 formed of a plurality of layers of electrolytically deposited metal with lubricating material interposed between said layers.

4. A hollow article having a shell formed 55 of a plurality of layers of electrolytically deposited metal with grease interposed between said layers.

5. A hollow article having a shell formed 60 of a plurality of layers of electrolytically deposited metal with non-conductive material interposed between said layers.

6. A hollow article having a shell formed 65 of a plurality of layers of electrolytically deposited metal with lubricating material interposed between said layers.

In testimony whereof, I have signed my name to this specification.

MATTHEW M. MERRITT.